

# United States Patent [19]

Sung et al.

[11] Patent Number: 4,609,377

[45] Date of Patent: Sep. 2, 1986

[54] AMINATED POLYISOPROPOXYLATED POLYETHOXYLATED ALKYLPHENOL AND ETHANOL/GASOLINE BLEND COMPOSITION CONTAINING SAME

[75] Inventors: Rodney L. Sung, Fishkill, N.Y.; Wheeler C. Crawford, Houston, Tex.

[73] Assignee: Texaco Inc., White Plains, N.Y.

[21] Appl. No.: 784,299

[22] Filed: Oct. 7, 1985

[51] Int. Cl.<sup>4</sup> ..... C10L 1/22

[52] U.S. Cl. ..... 44/56; 44/53; 44/72; 44/78; 252/392; 252/393; 252/148

[58] Field of Search ..... 44/53, 56, 78, 72; 252/148, 392, 393

## [56] References Cited

### U.S. PATENT DOCUMENTS

2,219,859 10/1940 White ..... 44/56  
4,207,076 6/1980 Boue et al. ..... 44/56  
4,207,077 6/1980 Boue et al. ..... 44/56  
4,252,746 2/1981 Kwong ..... 44/72

4,444,566 4/1984 Crawford et al. ..... 44/72  
4,541,945 9/1985 Anderson et al. ..... 252/148

Primary Examiner—Mrs. Y. Harris-Smith  
Attorney, Agent, or Firm—Robert A. Kulason; James J. O'Loughlin; Vincent A. Mallare

## [57] ABSTRACT

A novel fuel composition contains ethanol or gasohol, and, as a wear-corrosion-inhibiting additive, an aminated polyisopropoxylated polyethoxylated alkylphenol



wherein R is a (C<sub>5</sub>—C<sub>30</sub>) alkyl, alkaryl, aralkyl, aryl, or cycloalkyl group, x is a numeral of about 5 to about 30, and y is a numeral of about 1 to about 20.

11 Claims, No Drawings

AMINATED POLYISOPROPOXYLATED  
POLYETHOXYLATED ALKYLPHENOL AND  
ETHANOL/GASOLINE BLEND COMPOSITION  
CONTAINING SAME

BACKGROUND OF THE INVENTION

This invention relates to alcohol products particularly characterized by decreased ability to corrode and wear metal surfaces with which they come into contact.

As is well known to those skilled in the art, alcohols such as ethanol may corrode metal surfaces with which they come into contact. This is particularly true of crude or commercially available ethanols which undesirably contain acidic components commonly acetic acid. In the case of fermentation alcohols, acetic acid may be present in an amount of 0.003 wt.%–0.005 wt.% of the alcohol; and this may be responsible for the fact that the alcohol causes serious corrosion and wear problems.

It is an object of this invention to provide a novel process for decreasing the corrosion and wear of alcohol compositions. Other objects will be apparent to those skilled in the art.

SUMMARY OF THE INVENTION

The novel composition of this invention may comprises (i) a major portion of a fuel containing ethanol and (ii) gasoline in an amount of 0–50 volumes per volume of ethanol; and (iii) a minor effective wear-corrosion-inhibiting amount of, as a wear-corrosion-inhibiting additive, a nonionic surfactant of an aminated polyisopropoxylated polyethoxylated alkylphenol



wherein R is a (C<sub>5</sub>–C<sub>30</sub>) alkyl, alkaryl, aralkyl, aryl, or cycloalkyl group, x is a numeral of about 5 to about 30, and y is a numeral of about 1 to about 20.

DESCRIPTION OF THE INVENTION

The fuel for internal combustion engines which may be treated by the process of this invention may contain (i) ethanol and (ii) gasoline in an amount of 0–50 volumes per volume of ethanol. The fuel may be an alcohol-type fuel containing little or no hydrocarbon. Commercially available mixtures may be employed. Illustrative of one such commercially available mixture may be a simulated Brazilian ethanol fuel (SBEF) having the typical analysis provided below in Table I.

TABLE I

| Component              | Parts  |
|------------------------|--------|
| ethanol                | 3157.2 |
| methyl isobutyl ketone | 126.3  |
| acetic acid            | 0.256  |
| methyl alcohol         | 0.24   |
| isopropyl alcohol      | 0.2    |
| n-propyl alcohol       | 0.162  |
| ethyl acetate          | 0.2    |

The fuels which may be treated by the process of this invention include gasohols which may be formed by mixing 90–95 volumes of gasoline with 5–10 volumes of

ethanol. A typical gasohol may contain 90 volumes of gasoline and 10 volumes of SBEF.

It is preferred that the fuels to be treated by the process of this invention be substantially anhydrous, i.e., that they contain less than about 0.3 v% water; preferably from about 0.0001 v% to about 0.05 v%, and more preferably about 0.04 v% water.

It is a feature of these fuels that they may undesirably contain acidic contaminants which they cause serious corrosion and wear problems. These contaminants are particularly evident when the ethanol is commercially available and contains therein *inter alia* acids concurrently produced as by fermentation processes for producing ethanol or acids which have been picked up during handling. Acetic acid is a common acid present in the commercially available alcohols produced by fermentation; and it may be present in amount of 0.003 wt.%–0.005 wt.% of the total of the ethanol.

In accordance with practice of the process of this invention, there may be added to the fuel a minor wear-corrosion-inhibiting amount of, as a wear-corrosion-inhibiting additive, a nonionic surfactant of an aminated polyisopropoxylated polyethoxylated alkylphenol



wherein R is a (C<sub>5</sub>–C<sub>30</sub>) alkyl, alkaryl, aralkyl, aryl, or cycloalkyl group, preferably a (C<sub>5</sub>–C<sub>12</sub>) alkyl group and more preferably a C<sub>9</sub> alkyl group; x is a numeral of about 1 to about 20, preferably about 1 to about 10 and more preferably about 9.5; and y is a numeral of about 1 to about 10, preferably about 1 to about 5 and more preferably about 1.

The aminated polyisopropoxylated polyethoxylated alkylphenol is available under the trademark AMINATED SURFONIC, and is manufactured by Texaco Chemical Company of Houston, Tex.

Illustrative of these compositions are those listed below in Table II, the first listed being the most preferred.

TABLE II

|      |                         |
|------|-------------------------|
| I.   | Aminated Surfonic N-95  |
| 50   |                         |
| II.  | Aminated Surfonic N-120 |
| 60   |                         |
| III. | Aminated Surfonic N-40  |
| 65   |                         |



off and replaced with 10 ml of distilled water. The bottle is shaken the sample is maintained for 3 hours at 90° F. The percent rust on the strip is determined visually. A second reading is taken after 6 days and further readings may be taken.

The inhibited alcohols of this invention, after 18 hours of the ISCT generally show a Rust and Corrosion rating below about 2-3% and frequently as low as trace-to-1%.

#### EXAMPLE VII

In this example, the reaction product of Example I (i.e., 100 PTB of additive) was added to 90 parts of simulated Brazilian ethanol fuel containing

| Component              | Parts  |
|------------------------|--------|
| ethanol                | 3157.2 |
| methyl isobutyl ketone | 126.3  |
| glacial acetic acid    | 0.256  |
| n-butyl alcohol        | 0.24   |
| isopropyl alcohol      | 0.2    |
| n-propyl alcohol       | 0.162  |
| ethyl acetate          | 0.2    |

Distilled water (10 parts) was then added and the 25 system was subjected to the ISCT. The iron strip was observed after 6 days.

#### EXAMPLE VIII

In this control Example, the system of Example II 30 was tested without an additive.

The results of the Iron Strip Corrosion Test were as shown below in Table V.

TABLE V

| Example | Rust & Corrosion Rating          |       |
|---------|----------------------------------|-------|
| VII     | Instant Invention                | Trace |
| VIII    | Simulated Brazilian Ethanol Fuel | 50%   |

From Table V above, it is apparent that the system of Example VII, prepared in accordance with the practice of this invention showed only a trace of rust and corrosion, whereas control Example VIII showed a 50% rust and corrosion which is unsatisfactory.

#### EXAMPLE IX

In this example, both the fuel composition of the instant invention as described above in Example VII, and a gasohol were subjected to the ISCT. The iron strip was observed after 30 days. The results of the ISCT were as shown below in Table VI.

TABLE VI

| Example | Rust & Corrosion Rating                                                   |       |
|---------|---------------------------------------------------------------------------|-------|
| VII     | Instant Invention                                                         | Trace |
| IX      | Gasohol (10% simulated Brazilian ethanol fuel and 90% unleaded base fuel) | 5-10% |

From Table VI above, it is apparent that the system of Example VII, prepared in accordance of this invention, showed only a trace of rust and corrosion, whereas the gasohol of Example IX showed a 5-10% rust and corrosion which is unsatisfactory.

Results comparable to those of Example VII may be obtained when there is added the polyisopropoxylated

polyethoxylated alkylphenols listed below in Table VII.

TABLE VII

| Example |                                                                                    |
|---------|------------------------------------------------------------------------------------|
| X.      | Aminated Surfonic N-120                                                            |
| 10      |  |
| XI.     | Aminated Surfonic N-40                                                             |
| 15      |  |
| 20      | XII. Aminated Surfonic N-95                                                        |
|         |  |

Results comparable to those of Example VI may be obtained if the fuel used is as shown below in Table VIII.

TABLE VII

| Example | Fuel                                       |
|---------|--------------------------------------------|
| XIII    | Gasohol (90 v % gasoline and 10 v % SBEF)) |
| XIV     | SBEF                                       |

Although this invention has been illustrated by reference to specific embodiments, it will be apparent to those skilled in the art that various changes and modifications may be made which clearly fall within the scope of this invention.

I claim:

1. A fuel composition for internal combustion engines comprising
  - (a) a major portion of a fuel containing (i) ethanol and (ii) gasoline in amount of 0-50 volumes per volume of alcohol; and
  - (b) a minor wear-corrosion-inhibiting amount of, as a wear-corrosion-inhibiting additive, nonionic surfactant of an aminated polyisopropoxylated polyethoxylated alkylphenol



wherein R is a (C<sub>5</sub>-C<sub>30</sub>) alkyl, alkaryl, aralkyl, aryl, or cycloalkyl group, x is a numeral of about 5 to about 30, and y is a numeral of about 1 to about 20.

2. The fuel composition of claim 1, wherein said fuel is a commercial ethanol.
3. The fuel composition of claim 1, wherein said fuel is a commercial ethanol containing acid.
4. The fuel composition of claim 1, wherein said fuel is a commercial ethanol containing acetic acid.

5. The fuel composition of claim 1, wherein said fuel  
is a gasohol.

6. The fuel composition of claim 1, wherein said fuel 5  
is substantially anhydrous.

7. The fuel composition of claim 1, wherein said fuel  
contains less than 0.3 v% water. 10

8. The fuel composition of claim 1, wherein said  
amine is 15



9. The fuel composition of claim 1, wherein said  
amine is 20

10. The fuel composition of claim 1, wherein said  
amine is 10



wherein y is a numeral of 1 to 2.

11. The fuel composition of claim 1, wherein said  
amine is 15



\* \* \* \* \*

30

35

40

45

50

55

60

65